

## UNITED STATES PATENT OFFICE

2,647,872

## GREASE COMPOSITION

Walter H. Peterson, Point Richmond, Calif., assignor to Shell Development Company, San Francisco, Calif., a Delaware corporation

No Drawing. Application January 27, 1950,  
Serial No. 140,973

11 Claims. (Cl. 252—28)

1

This invention is concerned with improved grease compositions. More particularly, it relates to greases gelled by the presence of inorganic gelling agents such as silica and containing a combination of additive materials for the purpose of improving the water-resistance characteristics of the greases.

Greases are known which contain as their gelling agents certain inorganic materials such as silica aerogels and the like. While these greases exhibit outstanding performance under high temperature conditions, when compared with ordinary soap greases, they also possess inherent sensitivity to destruction by the action of water. Thus, when such greases are used for lubricating purposes when water or water-vapor is present, they tend to separate into two phases, namely an oil phase and a hydrated silica phase with consequent destruction of the grease. A copending patent application by the present inventor, Serial No. 82,905, filed March 22, 1949, now Patent No. 2,573,650 describes the use of certain agents for improving the water-resistance of such greases. The agents described in this copending application are hydroxy-containing organic compounds, as more particularly defined hereinafter. While the use of these compounds improves the water-resistance of the subject greases to a marked extent, there has been room for considerable improvement in this respect.

It is an object of the present invention to provide improved inorganic gel greases. It is another object of the present invention to provide inorganic gel greases having a higher water-resistance than those heretofore produced. It is an additional object of the present invention to provide greases which not only exhibit outstanding resistance to the deleterious action of water, but which also exhibit minimum corrosion characteristics.

Now, in accordance with this invention, it has been found that the resistance of inorganic gel greases to deterioration by water is improved to an unexpected extent by the combined addition thereto of certain hydrophobic surface active hydroxyl-containing organic compounds together with certain succinic or succinamic acids, their anhydrides, esters or amides. Not only do these succinic acid derivatives enhance the water-resistance of the subject greases in an unexplained manner, but they impart improved corrosion characteristics to the greases as well without adversely affecting the grease structure.

The succinic and succinamic acids useful in the present compositions are those bearing alkyl and alkenyl substituents, having from 5 to 36

2

carbon atoms and preferably between 10 and 24 carbon atoms.

Alkylated succinic acids are most readily prepared by condensing maleic acid anhydride with individual olefins or mixtures of olefins, particularly monoolefins. The resulting alkenyl succinic acid anhydrides may then be hydrated to liberate the free succinic acids, which may be used as such for blending with the lubricating oil or which may first be hydrogenated to produce the saturated alkyl succinic acids. An illustrative method of preparing these substances is set forth in the Eichwald patent, U. S. 2,055,456. The term alkyl succinic acids as herein used refers to both the unsaturated as well as the saturated products obtained when condensing maleic acid anhydride and olefins, hydrating the product to liberate the free acids, and hydrogenating the latter, if desired.

As to the boiling limits of suitable olefins there appear to be no critical limitations affecting the ability to prevent corrosion of the alkyl succinic acids produced therewith. However, it is desirable that the olefins be capable of distillation without substantial decomposition for the purpose of purifying the olefins as well as of separating unreacted olefins from the succinic acids produced therewith. In general, therefore, it is preferred that the normal boiling points of the distillate fractions be above 250° C. but not greatly in excess of 400° C. Most olefins normally boiling below about 400° C. can be distilled readily, if not under normal, then under reduced pressures, without noticeable decomposition.

Suitable olefins to be used in the condensation reaction with maleic acid anhydride may be produced by cracking a heavy oil, preferably in the vapor phase, under conditions to yield maximum amounts of the desired high boiling olefins, or else low boiling olefins may be polymerized to yield higher boiling olefins. Of particular usefulness are the normal olefins obtained in the vapor phase cracking of wax at temperatures around 560° C., although branched olefins may be used. The olefins may be of either primary or secondary or tertiary type.

The condensation reaction is carried out by digesting maleic acid anhydride with the desired olefins or olefin fraction at an elevated temperature, preferably 150° C. to 250° C., and, if desired, in the presence of a mild condensing agent.

The following examples illustrate the preparation of typical preferred alkyl or alkenyl succinic acids.

Three hundred parts of a distillate fraction of vapor phase cracked wax, boiling between 280° C.

to 340° C., having a bromine number of 36 and an olefin content of about 60%, were heated in an autoclave with 33 parts of maleic acid anhydride for two hours at 220° C. The product of reaction was subjected to a vacuum distillation to separate unreacted distillate and small amounts of maleic acid anhydride from the condensate. Ninety seven parts of a residue were obtained having a saponification number of 345. This residue was then hydrated with an amount of water corresponding to the saponification number for one hour at 90° C., whereby the anhydrides were converted to the free acids. All parts were by weight.

It will be understood that the subject alkyl and alkenyl succinic or succinamic acids may be utilized in the form of their anhydrides, free acids, amides, and aliphatic esters. The amides are sometimes regarded as condensation products formed between the succinic acid derivative and an amine. Either monoamides or diamides of the succinic acid derivatives may be employed and, furthermore, the amides may be formed from monoaliphatic amines or from aliphatic polyamines. The di- and triamines as well as the hydroxy derivatives thereof have been found to be especially suitable for the formation of effective condensation products with succinic acid for use in the subject compositions.

The condensation products utilized in accordance with the present invention may be prepared by various methods, of which the following are exemplary.

Olefin hydrocarbons containing from 5 to 20 carbon atoms produced by the dehydration of the corresponding alcohols, or by the removal of hydrogen halide from the corresponding hydrocarbon halides, or by the polymerization of lower olefins such as propylene, butylene, isobutylene, the amylenes, and the hexylenes or mixtures thereof, are caused to react with an unsaturated dicarboxylic acid or anhydride under the influence of heat to produce the alkenyl dicarboxylic acid or anhydride. Suitable charge materials include maleic anhydride or acid, fumaric acid, citraconic anhydride or acid, itaconic anhydride or acid, mesaconic acid, glutaconic anhydride or acid, methyl itaconic anhydride or acid, and the like. Alternatively, the alkyl dicarboxylic acid or anhydride may be prepared by hydrogenation of the corresponding C<sub>5</sub> to C<sub>20</sub> alkenyl dicarboxylic acid or anhydride or by treating a dicarboxylic acid ester with an alkali metal alcoholate in alcohol to replace a hydrogen atom on the alpha carbon atom of the ester with an alkali metal atom, and then reacting this product with an alkyl halide to introduce the alkyl group and eliminate the alkali metal as alkali metal halide. The alkylated dicarboxylic ester may then be reduced to the acid or the anhydride. Another method for producing the C<sub>5</sub> to C<sub>20</sub> dicarboxylic acid or anhydride comprises treating an unsaturated dicarboxylic acid or anhydride with a hydrogen halide to obtain a halogenated, saturated dicarboxylic acid or anhydride, and then replacing the halogen atom on the alpha carbon atom with an alkyl group by treatment with an alkyl halide and a catalyst or an alkali metal.

The alkyl or alkenyl dicarboxylic acid or anhydride may then be reacted with a monoamine, diamine or polyamine to obtain a condensation product suitable as an additive for the subject greases. The amines may be employed in molar ratios ranging from 1 to 2, although higher ratios

are not detrimental. Molar ratios of 1.3 to 2 have given very good results in the production of the condensation products. The amines which are preferred for the condensation reaction are those containing from 2 to 18 carbon atoms, and may be exemplified by ethylene diamine, diethylene triamine, triethylene tetramine, 1-methyl ethylene diamine, 1-ethyl ethylene diamine, propylene diamine, butylene diamine, trimethyl trimethylene diamine, tetramethylene diamine, diaminopentane or pentamethylene diamine, diaminohexane, hexamethylene diamine, heptamethylene diamine, diamino-octane, decamethylene diamine, and the higher homologs up to 18 carbon atoms, phenylene diamine, the alkylated phenylene diamines having nuclear substituents such as methyl, ethyl, propyl, butyl, etc., naphthalene diamine, and the alkylated naphthalene diamines. The condensation reaction may be carried out by simply adding the diamine or polyamine to the alkyl or alkenyl dicarboxylic acid or anhydride at ordinary temperature (60° F. to 80° F.) and then stirring vigorously. As the condensation proceeds, the temperature of the reaction mixture rises to 150° F.-220° F., with the elimination of water produced by the condensation. The condensation products, when cooled to room temperature, range from viscous, yellowish liquids to solids. When the charge materials are themselves solids, the reaction may be initiated by the application of heat sufficient to render the reactants liquid and capable of being mixed and stirred.

In the preparation of the condensation product of a diamine with an amido carboxylic acid, the latter may first be formed by treating an alkyl or alkenyl dicarboxylic acid or anhydride with ammonia (for example, 28% aqueous ammonia) to form the ammonium salt of the amido carboxylic acid. This product, when acidified with a mineral acid, such as hydrochloric acid, yielded the amido carboxylic acid, which in turn may be condensed with a diamine by stirring the mixture at ordinary temperature, heat being liberated as the condensation proceeds. The reaction temperature may rise to 120° F.-220° F., and upon cooling, the condensation products range from extremely viscous, yellow-orange liquids to wax-like solids.

Condensation products also suitable for use in accordance with this invention may be prepared by reacting the acid esters of the alkyl and alkenyl dicarboxylic acids or the acid esters of the alkyl and alkenyl amide carboxylic acids with diamines or polyamines. The acid esters may be produced by reacting, for example, equimolar quantities of an alcohol with the acid or anhydride. The alcohols may be exemplified by methyl, ethyl, propyl, isopropyl, butyl, amyl, etc. The reactants may be heated to temperatures of the order of 300° F. and maintained at this temperature for 1 to 3 hours, and then distilled to recover the desired acid ester. Another method for preparing the acid esters consists in reacting, for example, equimolar quantities of the acid or anhydride and an alkali metal alcoholate by refluxing the mixture at an elevated temperature for 2 to 8 hours in the presence of a diluent such as benzene. After refluxing, the alkali may be removed by washing the product with mineral acid, and then separating the benzene by distillation, leaving the desired acid ester. To prepare the condensation product, equimolar quantities, for example, of a diamine and the acid ester are

mixed at ordinary temperature and then vigorously stirred. As the condensation progresses, the temperature may rise to 120° F.-180° F., and after cooling, there is obtained a condensation product which may range from a viscous oil to a solid. The following is a typical process for the preparation of suitable succinic acid derivatives:

Nonylene, dodecylene, and octadecylene were reacted, respectively, with maleic anhydride by heating at 400° F. in a closed system with no external pressure applied, for a period of 1 to 4 hours. Vacuum distillation of the reaction products yielded the respective nonenyl, dodecenyl, and octadecenyl succinic anhydrides, substantially free of unreacted monoolefins and maleic anhydride. Using equimolar proportions of the monoolefin and the maleic anhydride gave a 40% to 60% yield of the corresponding alkenyl succinic anhydrides, whereas using 4 moles of monoolefin to 1 mole of maleic anhydride gave substantially 100% conversion into the corresponding alkenyl succinic anhydride.

The alkenyl succinic anhydrides as above prepared were condensed with ethylene diamine by slowly adding 2 moles of the diamine to the respective anhydrides at room temperature with vigorous stirring. Reaction immediately occurred and the temperature of the reaction mixture rose to 150° F.-220° F., with the elimination of by-product water.

The preferred species of succinic acid derivatives include especially the alkenyl succinic acids wherein the alkenyl groups contain 10 to 24 carbon atoms such as dodecenyl succinic acids, hexadecenyl succinic acids, octadecenyl succinic acids as well as mixtures thereof, such as are obtained by the condensation of maleic acid with mixed olefin hydrocarbons.

As stated hereinbefore, these alkenyl succinic acids may be converted to alkyl succinic acids by hydrogenation, to produce the corresponding preferred series of alkyl succinic acids wherein the alkyl group contains 10 to 24 carbon atoms. Thus, this group includes such typical species as tridecyl succinic acid, pentadecyl succinic acid, heptadecyl succinic acid and homologs thereof.

The preferred classes of succinic anhydrides, succinamic acids and succinamic anhydrides correspond to the above alkyl and alkenyl succinic acids. For example, suitable members of these groups are octadecyl succinic anhydrides, octadecenyl succinamic acid and dodecenyl succinamic anhydride.

The esters are preferably those of aliphatic alcohol having from 1 to 24 carbon atoms such as the methyl esters of octadecenyl succinic acid, the 2-ethylhexyl esters of hexadecyl succinamic acid, and the dodecenyl esters of decenyl succinic acid.

The aliphatic hydroxy compound to be used in the subject compositions are those disclosed in the copending patent application referred to hereinbefore. The principal classes useful for protecting the greases described hereinafter are especially hydroxy fatty acids, monohydric alcohol esters of said acids, polyhydric alcohols, esters of glycols and glycerols with hydroxy fatty acids, or esters of any fatty acid with polyhydric alcohol if the latter is only partially esterified, and natural products or modified natural products containing these types of compounds. It will be understood that other specialized groups of compounds meet the limitations given in the statement with the invention, but that these

groups are preferred due to their availability and effectiveness.

The text by A. W. Ralston "Fatty Acids and Their Derivatives," John Wiley & Sons, Inc., 1948, describes the more important types of hydroxy fatty acids and their esters which have been found to be useful in the present invention. The preferred hydroxy fatty acids useful for increasing the water-resistance of silica greases and the like include especially hydroxy stearic acids, and more particularly, 12-hydroxy stearic acid. Other homologs have been found to be effective as well such as stearic acids having hydroxy substituents in the 9, 10 or 11 positions. Polyhydroxy compounds also are effective, such as 9,10-dihydroxy stearic acid, 3,12-dihydroxy palmitic acid or 9,10,16-trihydroxy palmitic acid. While the saturated acids are preferred, those containing olefinic or acetylenic linkages may be used if available. These include such acids as 12-hydroxy ricinoleic acid, 19-hydroxy nonadecanoic acid and wool wax acids.

The hydroxy fatty acid glycerides which may be used in accordance with this invention are preferably the glycerides of fatty acids containing 8 or more carbon atoms and 1 or more hydroxyl radicals which are separated from the carboxyl group by at least one carbon atom. The preferred form of the material, due to availability and cost, is hydrogenated castor oil. Other glycerides of hydroxy fatty acids are effective for the present purpose such as glycerides of the hydroxy fatty acids produced by catalytic oxidation of hydrocarbon oils and waxes which have been extracted and fractionated to a desirable molecular weight range.

Partial esters of polyhydric alcohols and partial ethers of polyhydric alcohols are effective waterproofing agents for use in the present compositions. The preferred type of esters falling within this class include monoesters of glycerol wherein the ester radical contains at least 8 carbon atoms. A typical member of this class is glycerol monostearate. Ethers of glycerol containing 8 or more carbon atoms in the ether radical are exemplified by the monodecyl ether of glycerol.

The esters of monohydric alcohols with hydroxy fatty acids have been found to be effective water-proofing agents. Preferably, the esters are formed from alcohols having from 4 to 16 carbon atoms such as butyl, octyl and dodecyl alcohols together with hydroxy fatty acids such as those described above. A particularly effective member of this series is the butyl ester of 12-hydroxy stearic acid.

Glycols having at least 8 carbon atoms in the molecule also are suitable. Specific members of this class include octane diol, 1,4-dodecane diol, 1,2-decane diol and 1,10-decane diol. It is a preferred practice to apply glycols having widely spaced hydroxyl groups since it has been noted that glycols having hydroxyl groups attached to adjacent carbon atoms soften the grease to a certain extent, but glycols having widely spaced hydroxyl groups do not affect the grease in this manner. The lower polymers of alkylene glycols such as polyethylene glycol and polymethylene glycol are suitable water-proofing agents. The molecular weight of these polymers should be at least about 200 and preferably not more than about 800. Polyalkylene glycols having one of the end hydroxyl groups in the form of an ether or ester may be used as well. A typical member of this class is the monobutyl ether of tetraethylene glycol.

Higher molecular weight monohydric alcohols may be used such as octyl, decyl, dodecyl, stearyl and similar aliphatic monohydric alcohols. As was noted above, the corresponding mercapto compounds are effective for the present purpose and include especially higher molecular weight mercaptans such as dodecyl mercaptan.

The amounts of hydroxy compound and of succinic acid derivatives should vary from about 10 to 70% by weight of the gel and preferably is present in an amount between 20 to 50%. Based on the total grease the amounts of the additives are between 0.5 to 10%, preferably 1 to 5%. The effective amount of hydroxy compound required for improving the water-resistance of the greases described will vary with a number of factors; these include the molecular weight of the compound, the number of effective active groups such as hydroxyls, the amount of silica or other gel to be protected, and the surface area of said gel. The latter will depend upon the preparation of the gel and its subsequent grinding or reduction in particle size. The amount of silica or other gel will depend upon the grease consistency required. Ordinarily stated in terms of equivalence of effective hydroxyls it has been ascertained that from about .03 to about .10 equivalent of hydroxyls per 100 grams of silica gel provide excellent water protection for the greases. Preferably, the hydroxyl equivalent is between .05 to .08 per 100 grams of silica. The equivalent value is determined by dividing the molecular weight of a given hydroxy compound by the number of effective hydroxyl groups in the molecule.

The oil component of the subject grease compositions may be described broadly as an oleaginous vehicle which includes the conventional mineral lubricating oils, the synthetic lubricating oils prepared by cracking and polymerizing products of the Fischer-Tropsch process and the like; or a synthetic oleaginous compound within the lubricating oil viscosity range. The synthetic oleaginous compounds are those which possess lubricating characteristics or to which such characteristics may be imparted and may be substituted in whole or in part for the conventional mineral lubricating oils. Examples of these compounds are the aliphatic dicarboxylic acid esters such as the alkyl esters of sebacic acid, the high molecular weight aliphatic ethers as n-hexyl ether and the aromatic acid esters such as the alkyl esters of benzoic or phthalic acids. Other suitable synthetic lubricants include organic phosphates such as tricresyl phosphate, tributyl phosphate and mixed phosphates such as butyl dibenzyl phosphate. A special class of lubricants comprise the silicon oils which ordinarily require modification by the presence of a secondary lubricant or the use of lubricity imparting additives such as extreme pressure additives.

The agents which may be employed for the formation of greases in the oily fluids defined above include inorganic gels such as silica gel and other gels of inorganic oxides, hydroxides, sulfides and the like. It has been found to be substantially essential that the gels be used in a non-shrunken state such as may be obtained in the so-called "aerogel formation." Other means will be described hereinafter whereby gels suitable for use in the formation of greases may be prepared by other processes than aerogel formation. Typical aerogel greases are described in a patent to Kistler, U. S. 2,260,625. Other aerogels which are useful include magnesia, alumina, calcium oxide and the like. Hollow spheroidal gels, such

as those described by E. L. Largent in U. S. Patent 2,449,253, may be used in grease compositions.

One disadvantage which has been noted with respect to aerogels is their high bulk density. In accordance with one phase of the present invention, a means has been found for reducing the bulk density of aerogels and at the same time maintaining their ability to form greases with oleaginous components. This process comprises wetting the aerogel prepared after the manner described by Kistler with organic solvents such as acetone and isopentane. Other solvents comprise alcohols such as butyl alcohol, aldehydes such as acetaldehyde and similar low-boiling liquids having no solvent action on the aerogel and no chemical reaction therewith. The process comprises wetting the aerogel with a sufficient amount of the solvent such as acetone at room temperature and removing the solvent by warming or by the use of vacuum. The untreated aerogel has been found to be difficult to handle due to its high bulk density, while the treated aerogel appears to be in a more readily usable form resembling porous brittle aggregate lumps which are easily crushed to a powder.

The classes of polyvalent metal oxides and hydroxides forming gels are well known and do not require extensive discussion. The oxides and hydroxides of silicon, aluminum, chromium, copper, iron, manganese, titanium, nickel, calcium, germanium, molybdenum, thorium, tin and lead, and the like.

One of the means for preparing greases from inorganic gels without resorting to aerogel formation comprises dispersing an alcoholate or ester of the same group of metallic substances recited above in the lubricating medium and subsequently hydrolyzing to form the gel in situ, finally removing alcohol or other non-metallic products of the hydrolysis. This method inherently entails the advantage of avoiding aerogel formation and at the same time ensures the preparation of smooth, evenly dispersed greases having uniform structure.

A third method for the preparation of inorganic greases comprises formation of the hydrogel by well known processes commencing with an inorganic salt such as aluminum sulfate. By treatment of the salt dissolved in water with an agent such as ammonia, the hydrogel may be prepared and subsequently dehydrated by azeotropic distillation in the presence of a lower boiling alcohol such as ethanol. The alcohol suspension of the gel is then transferred to the lubricating oil medium after which alcohol is removed by distillation, preferably in vacuum. Upon removal of the alcohol and subsequent milling, a grease structure results wherein the inorganic gel is uniformly dispersed throughout the lubricating medium.

Effective amounts of gelling ingredients ordinarily are from about 1 to about 20% by weight of the oleaginous base. Preferably, the amount of gelling agent is from about 2 to 10% by weight of the oleaginous base.

The greases may be prepared as described above, either by separate preparation of the non-shrunken gel or by formation of the gel in the presence of the oil. The addition of waterproofing hydroxy compounds such as those described hereinbefore is preferably carried out subsequent to grease formation. It has been found that the degree of water-proofing for a given amount of the hydroxy compound is substantially greater if addition is effected at this stage rather

than prior to grease formation. However, effective water-proofing has been found to take place by initially dissolving the hydroxy compound in the oily medium and subsequently dispersing or forming the gel therein.

An additional type of inorganic gel grease which may be improved according to the present invention comprises greases gelled by the presence of organophilic clays and the like. The clays to be used in the present instance comprise those which have been treated with organic cationic surface active agents such as quaternary ammonium salts so as to destroy their inherent hydrophilic nature and to impart organophilic characteristics thereto. The essential preparation of 15 greases of this character comprise dispersing a swelling type of bentonite in water to form a hydrosol and adding 10 to 50% by weight of an ammonium salt such as dicetyl methyl ammonium chloride which causes the formation of a hydrogel wherein either absorption or ion exchange reaction has occurred so that a closely bonded composition of the bentonite and ammonium salt has resulted. The ammonium compound treated clay may then be incorporated directly with oil by milling together with simultaneous or subsequent heating for the removal of water. This method of direct transfer from a hydrogel into oil with the formation of grease 20 omitting any intermediate organogel formation or drying step is one which has been found to be highly desirable from an economic standpoint. While the addition of substituted succinic acids to the resulting greases has been found to result in improved water-resistance thereof, it is desirable to add as well one of the hydroxy-containing, surface active organic compounds as detailed above. Clays which are useful for the present purpose include especially montmorillonite such as the Wyoming bentonites or hectorite. While the swelling type of clays are those most highly desired, it is possible to prepare greases from the non-swelling type of clays, although larger amounts will be necessary to prepare a grease of a given penetration.

Summarizing the compositions described hereinabove, the preferred greases will contain the following ranges of proportions of their ingredients:

|                          | Per cent by weight of composition |
|--------------------------|-----------------------------------|
| Lubricating oil          | 60-98                             |
| Inorganic gelling agent  | 1-20                              |
| Hydroxy additive         | 1/2-10                            |
| Succinic acid derivative | 1/2-10                            |

It has been found that while the above ranges of ingredients are satisfactory in most instances, a clearer description may be made by reference of the ratio of hydroxy additive and succinic acid derivative based on the inorganic gel rather than upon the total grease composition. Hence, preferred compositions are those containing up to 20% of the inorganic gel based on the total grease and also containing 1 to 50% by weight of the inorganic gel of both the hydroxy-containing surface active agent and of the succinic acid derivative.

The following examples illustrate the advantages to be gained from the present compositions:

#### Example I

A mineral lubricating oil was milled with 5% by weight of a silica alcogel prepared by displacement of water from a silica hydrogel. During

the milling operation, 2.4% of the triglyceride of 12-hydroxy stearic acid were added to the mixture and the ingredients were milled to form a grease. A similar grease was prepared which 5 contained none of the glyceride additive. Following the milling operation, the greases were heated for a period of about one hour at a temperature of about 150 to 210° C. The grease containing only silica and lubricating oil disintegrated rapidly in the presence of boiling water. A sample of the grease prepared with silica and lubricating oil was modified by the addition of 1% by weight of the grease of octadecenyl succinic acids. This grease likewise disintegrated rapidly in the presence of boiling water. The silica grease containing the glyceride additive exhibited satisfactory resistance to boiling water. A fourth grease which contained the same amounts of both the glyceride additive and of octadecenyl succinic acids also showed satisfactory stability in the presence of boiling water. The four greases described above were then subjected to a roll stability test under the following conditions: 10 74 g. of the grease and 14 g. of water were rolled in a Shell Roll Tester (reference) and periodically tested until the grease reached a micro penetration of 230. It was found that the silica grease containing no additives failed almost at once. The silica grease containing only octadecenyl succinic acids failed in about one hour. The grease containing the glyceride additive failed in 20 12 hours, while the grease containing both additives lasted for 52 hours before failure.

#### Example II

35 Silica hydrogel was treated with aluminum sulfate to form a silica alumina hydrogel (composition). A 5% grease was prepared from the present silica alumina hydrogel by dehydrating the hydrogel with an ethyl alcohol, incorporating the organogel in mineral oil and evaporating off the alcohol. Three greases were prepared: Grease A contained no additives. Grease B contained 2% by weight of the triglyceride of 12-hydroxy stearic acid. Grease C was the same as 40 Grease B, but in addition contained 1% by weight of octadecenyl succinic acids. Each of the three greases contained 5% by weight of the silica alumina gel. For comparison two of the greases from Example I also were tested. Sample D was the grease from Example I containing the glyceride of 12-hydroxy stearic acid and sample E was the grease from Example I containing both the glyceride and octadecenyl succinic acid. The 45 greases described herewith were tested by smearing a layer of the grease on a steel strip which was then immersed in water contained in a test tube. The tube was placed in a steam bath and observed periodically for oil separation. The figures given in the table below represent the heating time in hours necessary to cause oil separation.

| Sample | Composition                                       | Hours under Heating |
|--------|---------------------------------------------------|---------------------|
| A      | Silica alumina                                    | 1.                  |
| B      | Silica alumina+glyceride                          | 16.                 |
| C      | Silica alumina+glyceride+succinic acid derivative | greater than 31.    |
| D      | Silica+glyceride                                  | 1.                  |
| E      | Silica+glyceride+succinic acid derivative         | 5.                  |

#### Example III

When greases are prepared by dispersing 5 parts by weight of the listed gelling agents, 1 part

## 11

by weight of the succinic acid derivative and 2 parts by weight of the surface active agent and 92 parts by weight of the mineral lubricating oil, the compositions which result are found to have excellent resistance to the action of hot water. If the surface active agent is omitted from any of the compositions, the grease which is formed from the remaining three components is found to be extremely sensitive to the action of cold water and to disintegrate immediately when contacted with hot water. Greases containing the gelling agents, mineral oil and surface active agent while showing moderate resistance to the action of cold water are quickly disintegrated in the presence of hot water.

| Sample | Gelling Agent | Succinic Acid Derivative                   | Surface Active Agent       |
|--------|---------------|--------------------------------------------|----------------------------|
| 1..... | Alumina       | Methyl ester of octadecenyl succinic acid. | 12-hydroxy stearic acid.   |
| 2..... | Silica        | Hexadecenyl succinamic acid.               | 1, 2-decamethylene glycol. |
| 3..... | do            | Dodecenyl succinic anhydride.              | Stearyl alcohol.           |

## Example IV

A grease was prepared containing 6% by weight of silica alcogel, 1% by weight of glycerol monostearate and 1% by weight of octadecenyl succinic acid. A similar grease was prepared omitting octadecenyl succinic acid. The first grease was found to have a hot water stability three times as great as that of the second grease.

I claim as my invention:

1. A grease composition comprising a mineral lubricating oil, 2-10% by weight of silica gel having a structure substantially that as originally formed, 1-5% by weight of 1,2-decamethylene glycol, and 1-5% by weight of hexadecenyl succinamic acid.

2. A grease composition comprising a mineral lubricating oil, 2-10% by weight of silica gel having a structure substantially that as originally formed, 1-5% by weight of a glyceride of 12-hydroxy stearic acid, and 1-5% by weight of octadecenyl succinic acid.

3. A grease composition comprising a mineral lubricating oil, 1-20% by weight of an inorganic oxide gel having a structure substantially that as originally formed, 0.5-10% by weight of a hydrophobic alkylene glycol having at least 8 carbon atoms and 0.5-10% by weight of a C<sub>5</sub>-36 alkenyl succinamic acid.

4. A grease composition comprising a mineral lubricating oil, 1-20% by weight of a silica gel having a structure substantially that as originally formed, 0.5-10% by weight of a glyceride of 12-hydroxy stearic acid, and 0.5-10% by weight of an octadecenyl succinic acid.

5. A grease composition comprising a mineral lubricating oil, 1-20% by weight of an inorganic oxide gel having a structure substantially that as originally formed, 0.5-10% by weight of an ester of a hydroxy fatty acid having at least 8 carbon atoms, and 0.5-10% by weight of an alkenyl succinic acid having at least one alkenyl group of 10 to 24 carbon atoms.

6. A grease composition comprising a mineral lubricating oil, 1-20% by weight of an inorganic oxide gel having a structure substantially that as originally formed, 0.5-10% by weight of a hydroxy fatty acid having at least 8 carbon atoms, and 0.5-10% by weight of an alkyl succinic acid

## 12

having at least one alkyl substituent of 10 to 24 carbon atoms.

7. A grease composition comprising a lubricating oil, 1-20% by weight of an originally hydrophilic inorganic gelling agent capable of forming a grease structure in said oil, 0.5-10% by weight of a hydroxy-containing hydrophobic surface-active agent of the groups consisting of hydroxy fatty acids, aliphatic alcohols having at least 8 carbon atoms per molecule, aliphatic esters of said acids and of said alcohols wherein each ester molecule contains at least 1 hydroxyl group, and mixtures of the same and 0.5-10% by weight of an alkyl succinic acid bearing at least one hydrocarbon group having from 5 to 36 carbon atoms.

8. A grease composition comprising a lubricating oil, 1-20% by weight of an originally hydrophilic inorganic gelling agent capable of forming a grease structure in said oil, 0.5-10% by weight of a hydroxy-containing hydrophobic surface-active agent of the groups consisting of hydroxy fatty acids, aliphatic alcohols having at least 8 carbon atoms per molecule, aliphatic esters of said acids and of said alcohols wherein each ester molecule contains at least 1 hydroxyl group, and mixtures of the same and 0.5-10% by weight of an alkenyl succinic acid bearing at least one hydrocarbon group having from 5 to 36 carbon atoms.

9. A grease composition comprising a lubricating oil, 1-20% by weight of an originally hydrophilic inorganic gelling agent capable of forming a grease structure in said oil, 0.5-10% by weight of a hydroxy-containing hydrophobic surface-active compound of the groups consisting of hydroxy fatty acids, aliphatic alcohols having at least 8 carbon atoms per molecule, aliphatic esters of said acids and of said alcohols wherein each ester molecule contains at least 1 hydroxyl group, and mixtures of the same and 0.5-10% by weight of an alkenyl succinic acid bearing at least one hydrocarbon group having from 5 to 36 carbon atoms.

10. A grease composition comprising a mineral lubricating oil, 2-10% by weight of an inorganic oxide gel capable of forming a grease structure in said oil, 1-10% by weight of 12-hydroxystearic acid and 1-5% by weight of an alkenyl succinic acid having an alkenyl group of 10 to 24 carbon atoms.

11. A grease composition comprising a mineral lubricating oil, 2-10% by weight of an inorganic oxide gel capable of forming a grease structure in said oil, 1-10% by weight of a hydrophobic hydroxy fatty acid and 1-5% by weight of an alkenyl succinic acid having an alkenyl group of 10 to 24 carbon atoms.

WALTER H. PETERSON.

## References Cited in the file of this patent

## UNITED STATES PATENTS

| Number    | Name           | Date          |
|-----------|----------------|---------------|
| 2,124,628 | Moser          | July 26, 1938 |
| 2,133,734 | Moser          | Oct. 18, 1938 |
| 2,260,625 | Kistler        | Oct. 28, 1941 |
| 2,445,936 | Butcosk        | July 27, 1948 |
| 2,491,441 | Butcosk et al. | Dec. 13, 1949 |